

## UNITED STATES PATENT OFFICE

2,389,523

BARIUM CALCIUM MAGNESIUM STEARATE  
GREASE

Frank A. Leyda, Berkeley, Calif., assignor, by  
mesne assignments, to California Research Cor-  
poration, San Francisco, Calif., a corporation  
of Delaware

No Drawing. Application November 2, 1943,  
Serial No. 508,749

8 Claims. (Cl. 252—39)

This invention relates to the preparation of lubricating greases and the greases produced thereby, particularly one which is waterproof, high melting and thermally reversible.

The three most commonly used bases for greases are soda, lime and aluminum soaps. Each type of grease made from these bases has certain advantages as well as disadvantages. Soda base greases have high melting points and are thermally reversible; i. e., on melting and then cooling to solidify, a soda base grease reverts to its original state. It does not break into an oil phase and a soap phase upon melting. However, due to the water solubility of the soda soaps, greases made from this material as a base lack waterproof qualities and will tend to emulsify with any moisture that may be present.

Lime or calcium base greases are waterproof, but melt at relatively low temperatures, about 200° F. Under these conditions they lose the water which is a minor but essential component of this type of grease and break into an oil phase and a soap phase. Thus, in addition to being low melting, which in itself is undesirable, lime base greases are not thermally reversible.

Aluminum base greases are waterproof but form a rubbery gel at about 200° F. Also, although aluminum base greases have an apparent melting point by the Ubbelohde or bulb methods as high as 250 to 300° F., it will be found that they will soften sufficiently to flow at temperatures of about 200° F. This may be demonstrated by placing a small sample of the grease upon a 6-mesh metal screen and heating it for several hours. Since many service conditions will impose a temperature of over 200° F. for prolonged periods, it is apparent that aluminum base greases are not high melting in the sense that soda base greases are high melting.

By way of improvement, it has been heretofore proposed to use barium base or mixed barium-calcium base greases in lieu of straight calcium base greases. Such greases have certain advantages, due chiefly to the barium base. Barium soaps, for example barium stearate, have the property of imparting to a grease a higher melting point than calcium soaps. At the same time the barium base grease retains the waterproof qualities of the calcium base material. Examples of these are described in United States Patents

Nos. 2,033,148 and 2,154,383 to Thomas F. Ott et al. Chiefly, such barium base greases include basic barium soap or a mixture of normal and basic barium soaps with petroleum oils of varying viscosity characteristics. Grease wherein the soap base is largely or entirely normal barium soap have a lower melting point than those in which the soap is of the basic variety. Mixed barium-calcium base greases are described in United States Patent No. 2,070,781 to L. C. Brunstrum et al. These are said to be superior not only to the lime or calcium base greases but also to the straight barium-base greases, in that they will not stiffen upon heating above 250° F. The mixed barium-calcium base greases are preferably used in conjunction with a partial ester of a polyhydric alcohol and a higher fatty acid, such as diglycol stearate. The combined effect of the mixed barium-calcium base and the partial ester is much greater than the effect of the barium-calcium base alone. This is particularly true of the anhydrous greases.

It is an object of the present invention to produce a grease having certain characteristics of calcium base greases and which combines several advantages and lacks several disadvantages of heretofore known greases.

It is a further and particular object of this invention to produce a grease which has a high melting point, is waterproof, and is thermally reversible and which is free from the objectionable features of heretofore known substitutes for calcium base greases.

Another object is to provide a method of producing an anhydrous grease which will be thermally reversible and will have improved resistance against melting at high temperatures.

These and other objects of this invention will be further apparent from the following description of a preferred embodiment together with several alternative compositions.

This invention comprehends broadly the utilization of a base comprising suitable soaps of barium, calcium and magnesium, said soaps including stearates, palmitates, a mixture of stearates and palmitates, or other fatty acids either occurring naturally or produced synthetically, such as those derived from the oxidation of petroleum wax. Strontium may be substituted in

part or in whole for the calcium in the base material.

In compounding greases according to the invention, the oil component will be selected and used from those petroleum oils which have hitherto been used in grease making. In a typical example, commercial stearic acid (a mixture of stearic and palmitic acids), barium hydroxide octahydrate, hydrated lime, magnesia and a mineral lubricating oil in quantity sufficient to render the mixture and the reaction produce freely fluid at an elevated temperature are stirred and heated in an autoclave at about 300 to 330° F. until saponification and intermixture are complete. After releasing the pressure, thereby flashing off a portion of the water, the autoclave is opened and the mixture heated further until substantially all of the water is driven off, after which sufficient mineral oil is added and stirred in to produce a grease of the desired consistency or hardness. After the mineral oil is added the grease is stirred and cooled to about 150° F. before drawing from the autoclave. It will be understood, however, that other procedures of compounding may be employed so long as the base comprises soaps of barium, calcium and magnesium and the saponified mixture is heated until substantially all the water is driven off to form an anhydrous product.

The term stearic acid is used in this description to designate both the comparatively pure acid and also the commercial product which may contain a substantial fraction, in some cases up to 40%, of palmitic acid.

The barium soap is preferably employed in greater amount than either of the other soaps and it is most advantageously used in an amount by weight exceeding the combined magnesium and calcium soaps. The preferred proportions of the various soaps are set forth in the table below:

| Per cent by weight of total soap |          |  |
|----------------------------------|----------|--|
| Barium soap                      | 60 to 80 |  |
| Calcium and/or strontium soap    | 10 to 30 |  |
| Magnesium soap                   | 10 to 20 |  |

As stated above, strontium may replace a part or all of the calcium soap, and the stearic acid radical may be replaced in part or entirely by the palmitic acid radical. Furthermore, other fatty acids may be used, such as the material sold under the trade-mark "Hydrex" derived from hydrogenated fish oil or similar oils and which consists of a mixture of saturated fatty acids in which the number of carbon atoms varies from about 14 to 22 or more. A typical average distribution would be as follows:

| Per cent |     |  |
|----------|-----|--|
| C-14     | 7   |  |
| C-16     | 32  |  |
| C-18     | 23  |  |
| C-20     | 23  |  |
| C-22+    | 15  |  |
|          | 100 |  |

The oil used in compounding the greases of this invention may be any conventional lubricating oil used in grease manufacture, including the medicinal white oils and low viscosity oils suitable for low temperature greases, but is preferably derived from Western type naphthenic oils having desirable solvent action and viscosity indices up to about 50.

It will be found that grease produced in ac-

cordance with this invention possesses a remarkable number of desirable properties. It is waterproof, like the calcium and aluminum base greases, but unlike both the latter it has a high melting point. Unlike aluminum base greases it does not gel to a rubbery state on heating. On the contrary, as it is heated to above the melting point it changes from a solid to a viscous liquid, and on cooling it again assumes the same solid form. Even repeated melting and solidification do not cause the oil and soap to separate, so that it is truly thermally reversible. Neither water nor any other substance besides the soaps and the oils is essential to its manufacture. Preferably, it is employed in an anhydrous form although a very small percentage of water may be present as is the case of substantially any form of grease.

Following are specific compositions of greases which have been found to be very desirable in their properties:

|    | Composition                                                                      | Example 1 | Example 2 |
|----|----------------------------------------------------------------------------------|-----------|-----------|
|    |                                                                                  | Percent   | Percent   |
| 25 | Stearic acid, percent by weight                                                  | 17.85     | 16.50     |
|    | Hydrated barium hydroxide                                                        | 7.52      | 6.95      |
|    | Hydrated lime                                                                    | 0.47      | 0.44      |
|    | Magnesia                                                                         | 0.20      | 0.18      |
| 30 | Acid treated naphthenic base mineral oil of viscosity 460 S. S. U. at 100° F.    |           | 75.93     |
|    | Solvent treated naphthenic base mineral oil of viscosity 350 S. S. U. at 100° F. | 73.98     |           |
|    |                                                                                  | 100.00    | 100.00    |
| 35 | A. S. T. M. penetration, 77° F.:                                                 |           |           |
|    | Unworked                                                                         | 125       | 158       |
|    | Worked                                                                           | 215       | 242       |
|    | Melting point, °F.                                                               | 205       | 250       |

40 In conclusion, it will be appreciated that the essential features of this invention appear to reside in the manufacture of an anhydrous grease which is waterproof, thermally reversible and of a high melting point, made from a mixture of barium, magnesium and calcium or strontium soaps with a mineral oil. Although specific examples of compositions, methods of compounding and the like have been given, it will be appreciated that modifications may be made which will not depart 45 from this invention so that all such modifications and changes as fall within the scope of the appended claims will be embraced thereby.

I claim:

1. A mixed base, anhydrous grease consisting 55 of mineral oil and soaps of barium, magnesium and at least one metal of the group consisting of calcium and strontium, said magnesium soap being present in proportions ranging from 10 to 20% of the soaps present so as to produce a thermally reversible grease.

2. A mixed-base, anhydrous grease consisting 60 of mineral oil and stearates and palmitates of barium, calcium and magnesium, said magnesium stearates and palmitates being present in such proportions as to produce a thermally reversible grease.

3. A mixed-base, thermally reversible grease consisting of mineral oil and a soap mixture, said soap mixture comprising about 10 to 20% 65 by weight of magnesium stearate, the other soaps comprising calcium and barium stearates, the barium stearate exceeding the combined calcium and magnesium stearate content.

4. A mixed base, anhydrous, thermally reversible grease comprising mineral oil and a soap mix-

ture, said soap mixture composed of 60 to 80% barium soap, 10 to 30% calcium soap and 10 to 20% magnesium soap.

5. A mixed base, anhydrous, thermally reversible grease comprising mineral oil and a soap mixture, said soap mixture composed of 60 to 80% barium soap, 10 to 30% strontium soap and 10 to 20% magnesium soap.

6. A mixed base, anhydrous, thermally reversible grease having approximately the following percentage composition by weight:

|                | Per cent |
|----------------|----------|
| Barium soap    | 18       |
| Calcium soap   | 4        |
| Magnesium soap | 3        |
| Oil            | 75       |

7. A mixed base, anhydrous, thermally reversible grease having approximately the following percentage composition by weight:

|                | Per cent |
|----------------|----------|
| Barium soap    | 18       |
| Strontium soap | 4        |
| Magnesium soap | 3        |
| Oil            | 75       |

8. A mixed-base, anhydrous thermally reversible grease comprising mineral oil and a soap mixture, said soap mixture composed of 60 to 80% barium soap, 10 to 20% magnesium soap, and about 10 to 30% of soap chosen from the group consisting of calcium and strontium soaps.

FRANK A. LEYDA.